

# UNITED STATES PATENT OFFICE.

MARCUS RUTHENBURG, OF LOCKPORT, NEW YORK.

## ORE-SEPARATING PROCESS.

933,491.

Specification of Letters Patent.

Patented Sept. 7, 1909.

No Drawing. Application filed January 6, 1908, Serial No. 409,535. Renewed July 31, 1909. Serial No. 510,681.

*To all whom it may concern:*

Be it known that I, MARCUS RUTHENBURG, of Lockport, in the county of Niagara and State of New York, have invented a certain new and useful Improvement in Ore-Separating Processes, whereof the following is a specification.

My improved process is adapted for the gravitational separation of hydrofuge ores and concentrates which will not gravitate in water. For instance, my process is applicable to the various sulfids and arsenids of copper, lead, zinc and iron which when crushed for concentration or separation from the gangue, form powdery slimes which, because of their peculiar surface repulsion, in jiggling or tabling with water either remain suspended in the water or float thereon, and in either case, are lost.

My invention is also applicable to separate the greasy complex or mixed concentrates of the ores of copper, zinc, lead, etc., which are produced by the "Elmore" process which consists in causing the crushed ore to absorb a thick oil and then floating it on a body of water in a vacuum chamber.

My invention is based upon the fact that the hydrofuge slimes of sulfids and arsenids aforesaid, which can not be compelled to gravitate in water are readily wetted by and gravitate in the lighter liquid distillates of petroleum; for instance, naphtha, benzin, kerosene, paraffin oil, or other liquid hydrocarbons, and, that the heavy oil residue in said "Elmore" concentrates, is soluble in said lighter oils, so that, in either case, the ore particles are separated by gravitation in such hydrocarbon liquid media, instead of floating thereon or being retained in suspension therein, as in water. Therefore, my process consists in surrounding hydrofuge ore or concentrate with a liquid medium other than water, and particularly a liquid hydrocarbon, in which the comminuted particles of the ore will gravitate, so that the separation of the different components of the ore is effected by gravitation without flotation in said liquid. Such separation

may be conveniently effected on a simple inclined concentrating table, like the "Wiffley" for instance.

Although I have described my invention as applicable to sulfids, arsenids, and concentrates produced by the "Elmore" process, it is to be understood that it is not restricted to such use.

I claim:

1. The described process of separating ore or concentrate particles of different specific gravity, which cannot be wetted in water, which consists in surrounding the same with a non-metallic liquid capable of wetting the surfaces of said particles so that they are separated by gravity without flotation in said liquid.

2. The described process of separating ore or concentrate particles of different specific gravity, which cannot be wetted in water, which consists in surrounding the same with an anhydrous non-metallic liquid capable of wetting the surfaces of said particles so that they are separated by gravity without flotation in said liquid.

3. The described process of separating ore or concentrate particles of different specific gravity, which cannot be wetted in water, which consists in surrounding the same with a liquid hydrocarbon capable of wetting the surfaces of said particles so that they are separated by gravity without flotation in said liquid.

4. The described process of separating ore or concentrate particles of different specific gravity, which cannot be wetted in water, which consists in surrounding the same with a liquid petroleum distillate capable of wetting the surfaces of said particles so that they are separated by gravity without flotation in said liquid.

In testimony whereof, I have hereunto signed my name at London, England, this twentieth day of December, 1907.

MARCUS RUTHENBURG.

Witnesses:

H. D. JAMESON,  
F. L. RAND.